

## UNITED STATES PATENT OFFICE

2,348,290

## STABILIZED MOTOR FUEL

Everett E. Gilbert, Elizabeth, N. J., assignor to  
 Tide Water Associated Oil Company, Bayonne,  
 N. J., a corporation of Delaware

No Drawing. Application March 28, 1941,  
 Serial No. 385,695

6 Claims. (Cl. 44—74)

The present invention relates to antioxidants for use in inhibiting the development of gums in gasolines and to compositions comprising gasolines normally tending to form gums in the presence of air, as when in storage, having incorporated therewith such antioxidants.

The invention derives from the discovery that certain alkyl substituted amino diphenyl amines, more specifically amino diphenyl amines in which one phenyl nucleus is amino substituted and the other phenyl nucleus is alkyl substituted, possess outstanding inhibitor properties for the stated purpose. Compounds of this class having amino groups in the 2,4 position as shown in the following formula:



and in which R is an alkyl substituent group, preferably of branched chain type, are especially suitable. In the general formula, R may, of course, be any suitable alkyl residue such as methyl, ethyl, propyl, butyl, amyl, etc. Such compounds are characterized by high and enduring activity in inhibiting the development of gums in motor fuels, relatively high gasoline solubility and satisfactory low water solubility, making them particularly effective inhibitors for use in the stated service. The data hereinbelow, resulting from extended study of these compounds, are illustrative of their inhibitive activity.

The test procedure followed that prescribed by the American Society for Testing Materials for indicating the gum stability of gasoline. This test (D-525) is the conventional and well known oxygen bomb accelerated oxidation method in which a comparison of the induction periods obtained with respective uninhibited and inhibited samples provides a measure of the antioxidant activity of tested compounds.

The compound employed as inhibitor in the test and falling within the class of compounds of this invention was 2,4 diamino, 4' tertiary amyl diphenyl amine.

In the foregoing table the gasoline samples all comprise sweetened cracked distillate cut to motor fuel boiling range. As is customarily the case, samples taken at different times or from different cracking units vary in their potential gum forming tendencies as evaluated by the conventional induction period criterion. This circumstance appears in the foregoing data. Special advantage of the inhibitors of this invention resides in the consistent improvement obtained with such varying original motor fuel samples. The invention is not limited to use with the illustrative type of motor fuel and extends generally to gasolines requiring stability improvement regardless of origin and method of manufacture. The compounds with which the invention is concerned may, and are intended to be, used in any desired or optimum inhibiting proportions.

## 20 I claim:

1. A composition comprising gasoline normally tending to oxidize in storage and an alkyl amino diphenyl amine effective to inhibit said oxidation.
2. A composition comprising gasoline normally tending to oxidize in storage and an alkyl 2,4 diamino diphenyl amine effective to inhibit said oxidation.
3. A composition comprising gasoline normally tending to oxidize in storage and an oxidation inhibiting proportion of a diphenyl amine in which one of the phenyl groups containing an alkyl substituent and the other phenyl group is amino substituted.
- 35 4. A composition comprising gasoline normally tending to oxidize in storage and an oxidation inhibiting proportion of a compound from the class represented by the formula



45 wherein R represents an alkyl group.

5. A composition comprising gasoline normally tending to oxidize in storage and an oxidation inhibiting proportion of a diphenyl amine in which one of the phenyl groups contains a branched chain alkyl substituent and the other phenyl group is amino substituted.

6. A composition comprising gasoline normally tending to oxidize in storage and a relatively small proportion of 4', tertiary amyl 55 2,4 diamino diphenyl amine.

EVERETT E. GILBERT.

| Gasoline sample | Inhibitor           | Induction period |
|-----------------|---------------------|------------------|
| A.....          |                     | Minutes          |
| A.....          | 0.52 mgs./100 c. c. | 184              |
|                 |                     | 210              |
| B.....          |                     | 200              |
| B.....          | 0.48 mgs./100 c. c. | 300              |
| C.....          |                     | 205              |
| C.....          | 0.65 mgs./100 c. c. | 301              |